



US01216838B2

(12) **United States Patent**  
Nakajima et al.

(10) **Patent No.:** US 12,168,838 B2  
(45) **Date of Patent:** Dec. 17, 2024

(54) **ELECTROLYTIC COPPER FOIL**

(71) **Applicant:** MITSUI MINING & SMELTING CO., LTD., Tokyo (JP)

(72) **Inventors:** Daisuke Nakajima, Ageo (JP); Mitsuyoshi Matsuda, Ageo (JP); Yasuji Hara, Ageo (JP); Mitsuhiro Wada, Ageo (JP)

(73) **Assignee:** MITSUI MINING & SMELTING CO., LTD., Tokyo (JP)

(\*) **Notice:** Subject to any disclaimer, the term of this patent is extended or adjusted under 35 U.S.C. 154(b) by 340 days.

(21) **Appl. No.:** 17/792,842

(22) **PCT Filed:** Jan. 14, 2021

(86) **PCT No.:** PCT/JP2021/001102  
§ 371 (c)(1),  
(2) Date: Jul. 14, 2022

(87) **PCT Pub. No.:** WO2021/153256

PCT Pub. Date: Aug. 5, 2021

(65) **Prior Publication Data**

US 2023/0044366 A1 Feb. 9, 2023

(30) **Foreign Application Priority Data**

Jan. 30, 2020 (JP) ..... 2020-013719

(51) **Int. Cl.**  
C25D 5/00 (2006.01)  
C25D 7/06 (2006.01)

(52) **U.S. Cl.**  
CPC ..... C25D 5/611 (2020.08); C25D 5/617 (2020.08); C25D 7/0614 (2013.01)

(58) **Field of Classification Search**

CPC ..... C25D 5/60; C25D 5/605; C25D 5/611; C25D 5/615; C25D 5/617  
See application file for complete search history.

(56) **References Cited**

U.S. PATENT DOCUMENTS

2016/0260981 A1 9/2016 Lee et al.  
2018/0298508 A1 10/2018 Lai et al.

FOREIGN PATENT DOCUMENTS

EP 0 675 213 10/1995  
JP H7-268678 10/1995  
(Continued)

OTHER PUBLICATIONS

JP 2015-028197 Machine Translation (Year: 2015).\*

*Primary Examiner* — Zachary M Davis

(74) *Attorney, Agent, or Firm* — GREENBLUM & BERNSTEIN, P.L.C.

(57) **ABSTRACT**

Provided is an electrodeposited copper foil having high smoothness and exhibiting high flexibility (particularly, high flexibility after annealing at 180° C. for 1 hour) suitable for a flexible substrate. This electrodeposited copper foil has an Rz of 0.1 to 2.0  $\mu\text{m}$  on at least one surface. In cross-sectional analysis by EBSD, a proportion of an area occupied by copper crystal grains satisfying the following conditions relative to an area of an observation field occupied by copper crystal grains is 63% or more. The conditions are as follows: i) (101) orientation; ii) an aspect ratio of 0.500 or less; iii)  $|\sin \theta|$  of 0.001 to 0.707, where  $\theta$  (°) is an angle between a normal line of an electrode surface of the electrodeposited copper foil and a major axis of the copper crystal grain; and iv) when the crystal is elliptically approximated, a length of a minor axis of 0.38  $\mu\text{m}$  or smaller.

5 Claims, 2 Drawing Sheets



(56)

**References Cited**

FOREIGN PATENT DOCUMENTS

|    |              |                |           |
|----|--------------|----------------|-----------|
| JP | 2006-052441  | 2/2006         |           |
| JP | 2015028197 A | * 2/2015 ..... | C25D 5/10 |
| JP | 2016-160503  | 9/2016         |           |
| JP | 2016-537514  | 12/2016        |           |
| JP | 2018-178261  | 11/2018        |           |
| WO | 2014/104233  | 7/2014         |           |
| WO | 2014/119355  | 8/2014         |           |

\* cited by examiner



FIG. 1

|             | Ex.7* | Ex.4* | Ex.5* | Ex.6* | Ex.8* | Ex.9* | Ex.10* | Ex.11 |
|-------------|-------|-------|-------|-------|-------|-------|--------|-------|
| TSAH        | 29.9  | 33.7  | 31.8  | 27.9  | 29.2  | 28.2  | 32.6   | 28.8  |
| POVLC       | 1.7%  | 5.0%  | 34.5% | 34.6% | 52.8% | 54.5% | 59.5%  | 62.6% |
| EBSD        |       |       |       |       |       |       |        |       |
| IQ+IPF (ND) |       |       |       |       |       |       |        |       |

  

|             | Ex.3  | Ex.1  | Ex.2  |
|-------------|-------|-------|-------|
| TSAH        | 21.3  | 22.4  | 24.1  |
| POVLC       | 63.3% | 70.8% | 72.0% |
| EBSD        |       |       |       |
| IQ+IPF (ND) |       |       |       |

TSAH: Tensile strength after heating  
 POVLC: Proportion of vertically long crystals

The symbol \* represents a comparative example.  
 A unit of the tensile strength after heating is kgf/mm<sup>2</sup>.

FIG. 2

## 1

## ELECTROLYTIC COPPER FOIL

## TECHNICAL FIELD

The present invention relates to an electrodeposited copper foil, particularly to an electrodeposited copper foil used for a flexible substrate.

## BACKGROUND ART

Known as an electrodeposited copper foil for a printed wiring board is a copper foil containing chlorine as low as possible (hereinafter, referred to as a chlorine-free copper foil). For example, Patent Literature 1 (JP2006-52441A) discloses a copper foil with a Cl content of less than 30 ppm in an unprocessed copper foil. Patent Literature 2 (JPH7-268678A) discloses an electrodeposited copper foil in which each peak value of X-ray diffraction intensities of (111) planes and (220) planes measured from the electrolysis end surface side satisfies a predetermined condition, and disclosed is manufacturing this electrodeposited copper foil by using a copper electrolyte with regulating a lead ion concentration to 3 ppm or less, a tin ion concentration to 6 ppm or less, a chloride ion concentration to 2 ppm or less, a silicon ion concentration to 15 ppm or less, a calcium ion concentration to 30 ppm or less, and an arsenic ion concentration to 7 ppm or less.

In addition, known technique is that a small amount of chloride ion is added into a copper plating solution during foil formation to attempt to improve characteristics from conventional chlorine-free copper foils. For example, Patent Literature 3 (JP2018-178261A) discloses an electrodeposited copper foil in which (a) brightness  $L^*$  value on an unroughened side is 75 to 90 based on the  $L^*a^*b$  color system and (b) a tensile strength is 40 kgf/mm<sup>2</sup> or more and 55 kgf/mm<sup>2</sup> or less. It is described that a low angle granular boundary (LAGB) measured by electron backscatter diffraction (EBSD) is preferably less than 7.0% in percentage. This literature describes manufacturing the electrodeposited copper foil by using a plating solution having a chloride ion concentration of 10 ppm, 15 ppm, or 20 ppm, and using a current density of 60 A/dm<sup>2</sup>, 70 A/dm<sup>2</sup>, or 80 A/dm<sup>2</sup> in an initial copper-plating process.

## CITATION LIST

## Patent Literature

- Patent Literature 1: JP2006-52441A  
 Patent Literature 2: JPH7-268678A  
 Patent Literature 3: JP2018-178261A

## SUMMARY OF INVENTION

For a copper foil used for a flexible substrate, differing from a copper foil used for a rigid substrate, flexibility that can be freely bended by external force is required. Some chlorine-free copper foils have a certain degree of smoothness and flexibility, but further improvement in smoothness and flexibility is required. Although a copper foil typically has a characteristic of reduce in a tensile strength to increase flexibility by annealing, an electrodeposited copper foil tends to have a relatively higher tensile strength, that is, lower flexibility, after annealing (for example, 180° C. for 1 hour) than a rolled copper foil. Thus, an electrodeposited copper foil having a significantly low tensile strength (that is, high flexibility) after annealing is desired. However, an

## 2

electrodeposited copper foil having a low roughness surface with ten-point average roughness  $Rz$  of 0.1  $\mu\text{m}$  or larger and 2.0  $\mu\text{m}$  or smaller has difficulty in regulating a tensile strength after annealing, and achievement of both smoothness and flexibility is not easy at present.

The present inventors have found that a higher proportion occupied by vertically long columnar crystals longitudinally extending in the foil thickness direction (hereinafter, referred to as vertically long crystals), as specified by cross-sectional analysis with electron backscatter diffraction (EBSD), can provide an electrodeposited copper foil having high smoothness given by a ten-point average roughness  $Rz$  of 0.1  $\mu\text{m}$  or larger and 2.0  $\mu\text{m}$  or smaller and at the same time exhibiting high flexibility (particularly, high flexibility after annealing at 180° C. for 1 hour) suitable for a flexible substrate.

Accordingly, an object of the present invention is to provide an electrodeposited copper foil having high smoothness and at the same time exhibiting high flexibility (particularly, high flexibility after annealing at 180° C. for 1 hour) suitable for a flexible substrate.

According to an aspect of the present invention, there is provided an electrodeposited copper foil having a ten-point average roughness  $Rz$  of 0.1  $\mu\text{m}$  or larger and 2.0  $\mu\text{m}$  or smaller on at least one surface,

wherein in cross-sectional analysis by electron backscatter diffraction (EBSD), a proportion of an area occupied by copper crystal grains satisfying all of the following conditions:

- (101) orientation;
- an aspect ratio of 0.500 or less;
- $|\sin \theta|$  of 0.001 or more and 0.707 or less, where  $\theta$  (°) is an angle between a normal line of an electrode surface of the electrodeposited copper foil and a major axis of the copper crystal grain; and
- when the crystal is elliptically approximated, a length of a minor axis of 0.38  $\mu\text{m}$  or smaller, relative to an area of an observation field occupied by copper crystal grains is 63% or more.

According to another aspect of the present invention, there is provided a flexible substrate, comprising the electrodeposited copper foil.

## BRIEF DESCRIPTION OF DRAWINGS

FIG. 1 is a graph indicating a relationship between proportion of vertically long crystals and tensile strength after heating in electrodeposited copper foils obtained in Examples 1 to 11.

FIG. 2 is cross-sectional EBSD images (IQ+IPF map (in ND direction) of the electrodeposited copper foils obtained in Examples 1 to 11.

## DESCRIPTION OF EMBODIMENTS

## Definitions

An “electrode surface” of an electrodeposited copper foil herein is referred to a surface that was contacted with a cathode during manufacture of the electrodeposited copper foil. A “deposit surface” of an electrodeposited copper foil herein is referred to a surface on which electrodeposited copper is deposited, that is, a surface that was not contacted with the cathode during manufacture of the electrodeposited copper foil.

## 65 Electrodeposited Copper Foil

A copper foil according to the present invention is an electrodeposited copper foil. This electrodeposited copper

foil has a ten-point average roughness  $R_z$  of 0.1  $\mu\text{m}$  or larger and 2.0  $\mu\text{m}$  or smaller on at least one surface. In cross-sectional analysis by electron backscatter diffraction (EBSD), the electrodeposited copper foil has a proportion of an area occupied by copper crystal grains satisfying all the conditions below of 63% or more relative to an area of an observation field occupied by the copper crystal grains, the conditions being as follows: i) (101) orientation; ii) an aspect ratio of 0.500 or less; iii)  $|\sin \theta|$  of 0.001 or more and 0.707 or less, where  $\theta$  ( $^{\circ}$ ) is an angle between a normal line of an electrode surface of the electrodeposited copper foil and a major axis of the copper crystal grain; and iv) when the crystal is elliptically approximated, a length of a minor axis of 0.38  $\mu\text{m}$  or smaller. As above, a higher proportion occupied by the vertically long columnar crystals longitudinally extending in the foil thickness direction (hereinafter, referred to as vertically long crystals), as specified by cross-sectional analysis with electron backscatter diffraction (EBSD), can provide an electrodeposited copper foil having high smoothness given by a ten-point average roughness  $R_z$  of 0.1  $\mu\text{m}$  or larger and 2.0  $\mu\text{m}$  or smaller and at the same time exhibiting high flexibility (particularly, high flexibility after annealing at 180 $^{\circ}$  C. for 1 hour) suitable for a flexible substrate.

As described above, although a copper foil typically has the characteristic that annealing results in a decreased tensile strength and an increased flexibility, an electrodeposited copper foil tends to have a relatively higher tensile strength, that is, a lower flexibility than a rolled copper foil after annealing (for example, 180 $^{\circ}$  C. for 1 hour). Thus, an electrodeposited copper foil having a significantly low tensile strength (that is, high flexibility) after annealing is desired. However, an electrodeposited copper foil having a low roughness surface with ten-point average roughness  $R_z$  of 0.1  $\mu\text{m}$  or larger and 2.0  $\mu\text{m}$  or smaller has difficulty in regulating a tensile strength after annealing, and achievement of both smoothness and flexibility is not easy at present. From this viewpoint, the electrodeposited copper foil of the present invention can conveniently achieve both the smoothness and the flexibility.

The electrodeposited copper foil has a ten-point average roughness  $R_z$ , on at least one surface, of preferably 0.1  $\mu\text{m}$  or larger and 2.0  $\mu\text{m}$  or smaller, more preferably 0.3  $\mu\text{m}$  or larger and 2.0  $\mu\text{m}$  or smaller, further preferably 0.3  $\mu\text{m}$  or larger and 1.8  $\mu\text{m}$  or smaller, particularly preferably 0.6  $\mu\text{m}$  or larger and 1.5  $\mu\text{m}$  or smaller, and most preferably 0.6  $\mu\text{m}$  or larger and 1.2  $\mu\text{m}$  or smaller. Such an electrodeposited copper foil having a low roughness surface is advantageous from the viewpoint of less rupture starting points. The "ten-point average roughness  $R_z$ " herein is measured in accordance with JIS-B0601:1982, and corresponds to  $R_{zjjs}$  in JIS-B0601:2001.

The electrodeposited copper foil also preferably has a ten-point average roughness  $R_z$  within the above range on both surfaces. That is, the electrodeposited copper foil has a ten-point average roughness  $R_z$ , on both the surfaces, of preferably 0.1  $\mu\text{m}$  or larger and 2.0  $\mu\text{m}$  or smaller, more preferably 0.3  $\mu\text{m}$  or larger and 2.0  $\mu\text{m}$  or smaller, further preferably 0.3  $\mu\text{m}$  or larger and 1.8  $\mu\text{m}$  or smaller, particularly preferably 0.6  $\mu\text{m}$  or larger and 1.5  $\mu\text{m}$  or smaller, and most preferably 0.6  $\mu\text{m}$  or larger and 1.2  $\mu\text{m}$  or smaller. Such an electrodeposited copper foil having low roughness surfaces on both the surfaces is advantageous from the viewpoint of less rupture starting points.

The electrodeposited copper foil in an unannealed original state has a tensile strength of preferably 56 kgf/mm<sup>2</sup> or more and less than 65 kgf/mm<sup>2</sup>, more preferably 57 kgf/mm<sup>2</sup> or more and 64 kgf/mm<sup>2</sup> or less, further preferably 59 kgf/mm<sup>2</sup> or more and 64 kgf/mm<sup>2</sup> or less, and most preferably 60 kgf/mm<sup>2</sup> or more and 64 kgf/mm<sup>2</sup> or less. The electrodeposited copper foil after annealing at 180 $^{\circ}$  C. for 1 hour has a tensile strength of preferably 15 kgf/mm<sup>2</sup> or more and less than 25 kgf/mm<sup>2</sup>, more preferably 15 kgf/mm<sup>2</sup> or more and 24.5 kgf/mm<sup>2</sup> or less, further preferably 16 kgf/mm<sup>2</sup> or more and 24.5 kgf/mm<sup>2</sup> or less, and particularly preferably 16 kgf/mm<sup>2</sup> or more and 24 kgf/mm<sup>2</sup> or less. Within the above range, the electrodeposited copper foil can exhibit high flexibility suitable for a flexible substrate when a thermal history is applied by annealing (for example, 180 $^{\circ}$  C. for 1 hour). Both of the tensile strength in an unannealed original state and the tensile strength after annealing are measured in accordance with IPC-TM-650 at a room temperature (for example, 25 $^{\circ}$  C.).

The electrodeposited copper foil of the present invention has a high proportion occupied by vertically long columnar crystals longitudinally extending in the foil thickness direction (hereinafter, referred to as vertically long crystals), as evaluated for a cross section thereof. This fine structure rich in the vertically long crystals contributes to both of the high smoothness of a ten-point average roughness  $R_z$  of 0.1  $\mu\text{m}$  or larger and 2.0  $\mu\text{m}$  or smaller and the high flexibility (particularly, the high flexibility after annealing at 180 $^{\circ}$  C. for 1 hour) suitable for a flexible substrate. The vertically long crystals are specified as satisfying the following conditions when a cross section of the electrodeposited copper foil is analyzed by electron backscatter diffraction (EBSD). The conditions are as follows:

- i) (101) orientation;
- ii) an aspect ratio of 0.500 or less;
- iii)  $|\sin \theta|$  of 0.001 or more and 0.707 or less, where  $\theta$  ( $^{\circ}$ ) is an angle between a normal line of an electrode surface of the electrodeposited copper foil and a major axis of the copper crystal grain; and
- iv) when the crystal is elliptically approximated, a length of a minor axis of 0.38  $\mu\text{m}$  or smaller.

Specifically, in cross-sectional analysis by EBSD, the electrodeposited copper foil of the present invention has a proportion of an area occupied by the copper crystal grains satisfying all the above conditions i) to iv) (that is, the proportion of the vertically long crystals), relative to an area of an observation field (for example, 10  $\mu\text{m}$  in width $\times$ 28  $\mu\text{m}$  in height) occupied by copper crystal grains, of 63% or more, more preferably 63% or more and 90% or less, further preferably 63% or more and 85% or less, particularly preferably 63% or more and 80% or less, and most preferably 63% or more and 75% or less. Within the above range, achieved is both of the high smoothness of a ten-point average roughness  $R_z$  of 0.1  $\mu\text{m}$  or larger and 2.0  $\mu\text{m}$  or smaller and the high flexibility (particularly, the high flexibility after annealing at 180 $^{\circ}$  C. for 1 hour) suitable for a flexible substrate. Here, the observation field with EBSD specifies a rectangular region of width $\times$ height satisfying a condition shown in Table 1.

TABLE 1

| EBSD<br>observation<br>field | Correspondence<br>to copper foil                      | Specific size                                                                                                                                                                                                                                                                                                                                                                                                                      |
|------------------------------|-------------------------------------------------------|------------------------------------------------------------------------------------------------------------------------------------------------------------------------------------------------------------------------------------------------------------------------------------------------------------------------------------------------------------------------------------------------------------------------------------|
| Width                        | Length in<br>thickness<br>direction of<br>copper foil | Distance from $E_0$ to $E_1$ in the thickness direction of the copper foil ( $E_1-E_0$ ) where: $E_0$ is a field end at a position 3 $\mu\text{m}$ apart from the electrode surface of the copper foil in the thickness direction; and $E_1$ is an opposite field end nearest to the depositing surface of the copper foil when the largest range of an observation field full of copper crystals is incorporated within one field |
| Height                       | Length in<br>surface direction<br>of copper foil      | 28 $\mu\text{m}$ in the surface direction of the copper foil                                                                                                                                                                                                                                                                                                                                                                       |

With specifying the width in the EBSD observation field, a position 3  $\mu\text{m}$  apart from the electrode surface of the copper foil in the thickness direction is specified as a reference position  $P_0$  (that is, a region within 3  $\mu\text{m}$  from the electrode surface of the copper foil in the thickness direction is excluded from the field). This is because such exclusion of the surface layer region on the side in which the copper crystal grains become relatively or excessively fine due to influence of the cathode (particularly the structure thereof) used during manufacture of the electrodeposited copper foil provides the EBSD observation field more representatively reflecting a major component in the thickness direction of the copper foil.

The EBSD analysis can be performed by subjecting the electrodeposited copper foil to a cross-section polisher (CP) process to form a polished cross section, and by EBSD-analyzing the polished cross section within an observation field with width $\times$ height shown in Table 1 by using an EBSD apparatus (SUPRA55VP, manufactured by Carl Zeiss Co., Ltd.) under SEM conditions of  $\text{Vacc.}=20$  kV,  $\text{Apt.}=60$   $\mu\text{m}$ , H.C. mode, Tilt=70°, and Scan Phase=Cu.

The proportion of the vertically long crystals can be determined based on the EBSD image through the following steps.

—Primary Extraction Based on the Condition i):

The EBSD image in the observation field is analyzed by using an EBSD analysis software (OIM Analysis 7, available from TSL solutions K. K.) to extract crystals orientating in  $(h, k, l)=(1, 0, 1)$  (see Examples below for detailed setting conditions). This procedure extracts a crystal grain region satisfying the above condition i).

—Secondary Extraction Based on the Conditions ii), iii), and iv):

Further extracted based on the data obtained from the primary extraction is a crystal satisfying all the conditions of: an aspect ratio of 0.500 or less; a gradient of a major axis  $|sin \theta|$  of 0.001 or more and 0.707 or less; and when the crystal grain is elliptically approximated, a length of a minor axis of 0.38  $\mu\text{m}$  or smaller (see Examples below for detailed setting conditions). A summed area ( $\mu\text{m}^2$ ) of the above

20 crystals is obtained as an area of the vertically long crystal grains. This procedure extracts a crystal grain region satisfying the above conditions ii), iii), and iv).

—Calculation of Proportion of Vertically Long Crystals:

Using the area  $S_{vc}$  ( $\mu\text{m}^2$ ) of the vertically long crystal grains obtained in the secondary extraction and an area  $S_{OA}$  ( $\mu\text{m}^2$ ) of the observation field, a proportion occupied by the vertically long crystal grains relative to the area occupied by the copper crystal grains is calculated with a formula of  $100 \times S_{vc}/S_{OA}$  to be specified as the proportion of the vertically long crystals (%) (see Examples below for setting conditions).

35 35 A thickness of the electrodeposited copper foil is not particularly limited, but preferably 5  $\mu\text{m}$  or more and 35  $\mu\text{m}$  or less, more preferably 7  $\mu\text{m}$  or more and 35  $\mu\text{m}$  or less, further preferably 9  $\mu\text{m}$  or more and 18  $\mu\text{m}$  or less, and particularly preferably 12  $\mu\text{m}$  or more and 18  $\mu\text{m}$  or less.

40 40 The electrodeposited copper foil is preferably subjected to surface treatment on one surface or on both surfaces. This surface treatment may be one commonly performed in 45 electrodeposited copper foils. Preferable examples of the surface treatment include roughening treatment, rust proofing treatment (for example, zinc plating treatment and zinc-alloy plating treatment such as zinc-nickel-alloy plating treatment), and silane coupling agent treatment. The electrodeposited copper foil may be provided as a form of a carrier-attached copper foil.

Manufacturing Method

55 55 The electrodeposited copper foil of the present invention can be manufactured by using a copper electrolyte (aqueous solution) with a copper (Cu) concentration, sulfuric acid ( $\text{H}_2\text{SO}_4$ ) concentration, and chlorine (Cl) concentration shown in Table 2, and by maintaining a bath temperature (temperature of the aqueous solution) at a temperature shown in Table 2 to perform electrodeposition at a current density shown in Table 2. That is, satisfying these conditions of the copper electrolyte composition, bath temperature, and current density can achieve a cross-sectional structure with the proportion of the vertically long crystals of 63% or more. 60 60 As a result, it is possible to manufacture the electrodeposited

copper foil having the high smoothness given by a ten-point average roughness  $R_z$  of 0.1  $\mu\text{m}$  or larger and 2.0  $\mu\text{m}$  or smaller on the deposited surface (or both of the deposited surface and the electrode surface) and at the same time exhibiting the high flexibility (particularly, the high flexibility after annealing at 180° C. for 1 hour) suitable for a flexible substrate. As shown in Table 2, the copper electrolyte used in this manufacturing method is desirably a chlorine-free electrolyte containing chlorine as low as possible.

<Proportion of Vertically Long Crystals and EBSD Cross-Sectional Analysis>

Four samples of the electrodeposited copper foil were overlapped to be laminated with an adhesive (LOCTITE®, manufactured by Henkel Japan Ltd.), and then an ultraviolet-curable resin was applied on the sample surface as a protecting layer. The sample was entirely coated with carbon, then subjected to cross-sectional process with broad argon ion beam (CROSS SECTION POLISHER® (CP),

TABLE 2

| Composition of aqueous solution (copper electrolyte) |                      |                             |                        |                   |                                  |
|------------------------------------------------------|----------------------|-----------------------------|------------------------|-------------------|----------------------------------|
|                                                      | Copper concentration | Sulfuric acid concentration | Chlorine concentration | Bath temperature  | Current density                  |
| Preferable range                                     | 30 g/L or higher     | 150 g/L or higher           | 0 m g/L or higher      | 31° C. or higher  | 35 A/dm <sup>2</sup> or higher   |
|                                                      | 50 g/L or lower      | 210 g/L or lower            | 5 m g/L or lower       | lower than 33° C. | 45 A/dm <sup>2</sup> or lower    |
| More preferable range                                | 35 g/L or higher     | 155 g/L or higher           | 0 m g/L or higher      | 31° C. or higher  | 37.5 A/dm <sup>2</sup> or higher |
|                                                      | 50 g/L or lower      | 210 g/L or lower            | 5 m g/L or lower       | lower than 33° C. | 45 A/dm <sup>2</sup> or lower    |
| Further preferable range                             | 40 g/L or higher     | 160 g/L or higher           | 0 m g/L or higher      | 31° C. or higher  | 40 A/dm <sup>2</sup> or higher   |
|                                                      | 50 g/L or lower      | 210 g/L or lower            | 5 m g/L or lower       | lower than 33° C. | 45 A/dm <sup>2</sup> or lower    |

## EXAMPLES

The present invention will be described in more specific with the following examples.

## Examples 1 to 11

## (1) Manufacture of Electrodeposited Copper Foil

A sulfuric acid-acidic copper sulfate solution (no chlorine was added) with a composition shown in Table 4 was used as the copper electrolyte. A plate-shaped electrode (surface roughness  $R_a=0.19 \mu\text{m}$  in accordance with JIS-60601:1982) made of titanium was used as a cathode, and a DSA (dimensionally stable anode) was used as an anode. Electrodeposition was performed at a bath temperature and at a current density shown in Table 4 to obtain an electrodeposited copper foil having a thickness of 18  $\mu\text{m}$ .

## (2) Evaluation of Electrodeposited Copper Foil

On the obtained electrodeposited copper foil, measurement of ten-point average roughness  $R_z$ , cross-sectional analysis by EBSD, and measurement of tensile strength were performed as follows.

<Measurement of Ten-Point Average Roughness  $R_z$ >

A ten-point average roughness  $R_z$  (corresponding to  $R_{zjjs}$  in JIS-60601:2001) on a deposited surface of the electrodeposited copper foil was measured by using a surface roughness measuring instrument (Surfcorder SE-30H, manufactured by Kosaka Laboratory Ltd.) in accordance with JIS-60601:1982 under conditions of  $\lambda_c$ : 0.8  $\mu\text{m}$ , reference length: 0.8 mm, and feeding speed: 0.1 mm/s. Table 4 shows results.

manufactured by JEOL Ltd.) (accelerating voltage: 5 kV) for 3 hours to obtain a polished cross section for EBSD measurement. With EBSD observation, carbon coating (1 flash) was performed. The polished cross section was EBSD-analyzed by using an EBSD apparatus (FE-SEM apparatus (SUPRA55VP, manufactured by Carl Zeiss Co., Ltd.) equipped with an EBSD measuring apparatus (Pegasus, manufactured by AMETEK, Inc.)) under SEM conditions of  $\text{Vacc.}=20 \text{ kV}$ ,  $\text{Apt.}=60 \mu\text{m}$ ,  $\text{H.C. mode}$ ,  $\text{Tilt}=70^\circ$ , and  $\text{Scan Phase}=Cu$ . The observation field in the EBSD was set to 10  $\mu\text{m}$  in width $\times$ 28  $\mu\text{m}$  in height (in accordance with the above conditions shown in Table 1). In the EBSD image in the observation field, an area occupied by copper crystal grains satisfying all of the following conditions (hereinafter, referred to as an area of vertically long crystal grains) was determined by the following primary extraction and secondary extraction. The conditions are as follows:

- (101) orientation;
- an aspect ratio of 0.500 or less;
- $|\sin \theta|$  of 0.001 or more and 0.707 or less, where  $\theta$  (°) is an angle between a normal line of the electrode surface of the electrodeposited copper foil and a major axis of the copper crystal grain; and
- when the crystal is elliptically approximated, a length of a minor axis of 0.38  $\mu\text{m}$  or smaller.

## —Primary Extraction Based on the Condition i)

The EBSD image in the observation field is analyzed by using an EBSD analysis software (OIM Analysis 7, available from TSL solutions K. K.) to extract crystals orientating in  $(hkl)=(101)$ . A specific procedure was as follows. In a screen of OIM Analysis 7, [All data], [Property], [Crystal Orientation], and  $[(h,k,l)=(1,0,1)]$  was selected. Then, a

value of [Deviation] was set to be less than 60, (h,k,l)=(1, 0,1) was selected in [Crystal Deviation], and then a value of [Derivation] was set to be less than 12 to extract [Grain data], that is, particle data. In this time, setting conditions of OIM Analysis 7 were as follows.

PCO [Copper, 0.000, 45.000, 90.000]<60

AND PCD [Copper, 1, 0, 1, 0, 0, 1]<12

—Secondary Extraction Based on the Conditions ii), iii), and iv)

Further extracted based on the data obtained in the above were crystals satisfying all the conditions of: an aspect ratio of 0.500 or less; a gradient of a major axis  $|\sin \theta|$  of 0.001 or more and 0.707 or less; and when the crystal grain is elliptically approximated, a length of a minor axis of 0.38

specimen. This specimen was set in a measuring apparatus (AGI-1KNM1, manufactured by SHIMADZU CORPORATION) to measure an original tensile strength at a room temperature (approximately 25° C.) in accordance with 5 IPC-TM-650 under conditions of tensile speed: 50 mm/min and full-scale test force: 50 N. Table 4 shows results.

<Measurement of Tensile Strength after Heating>

10 A sample of the electrodeposited copper foil after annealing at 180° C. for 1 hour was cut in a size of 10 mm×100 mm to obtain a specimen. A tensile strength of this specimen was measured under the same conditions as in the measurement of the original tensile strength to measure a tensile strength after heating. Table 4 shows results.

TABLE 4

|             | Manufacturing conditions                                    |                                      |                            |                                         | Electrodeposited copper foil  |                                            |                                          |                                         |
|-------------|-------------------------------------------------------------|--------------------------------------|----------------------------|-----------------------------------------|-------------------------------|--------------------------------------------|------------------------------------------|-----------------------------------------|
|             | Composition of copper electrolyte<br>(no chlorine is added) |                                      |                            |                                         | EBSD cross-sectional analysis |                                            | Tensile strength                         |                                         |
|             | Copper concentration<br>(g/L)                               | Sulfuric acid concentration<br>(g/L) | Bath temperature<br>(° C.) | Current density<br>(A/dm <sup>2</sup> ) | Rz<br>(μm)                    | Proportion of vertically long crystals (%) | Original state<br>(kgf/mm <sup>2</sup> ) | After heating<br>(kgf/mm <sup>2</sup> ) |
| Example 1   | 40                                                          | 160                                  | 31                         | 40                                      | 0.79                          | 70.8                                       | 58.9                                     | 22.4                                    |
| Example 2   | 50                                                          | 160                                  | 31                         | 45                                      | 1.23                          | 72.0                                       | 61.0                                     | 24.1                                    |
| Example 3   | 50                                                          | 210                                  | 31                         | 45                                      | 1.07                          | 63.3                                       | 63.3                                     | 21.3                                    |
| Example 4*  | 40                                                          | 110                                  | 39                         | 35                                      | 2.31                          | 5.0                                        | 42.4                                     | 33.7                                    |
| Example 5*  | 40                                                          | 160                                  | 35                         | 40                                      | 1.56                          | 34.5                                       | 45.4                                     | 31.8                                    |
| Example 6*  | 50                                                          | 210                                  | 35                         | 45                                      | 1.68                          | 34.6                                       | 56.7                                     | 27.9                                    |
| Example 7*  | 50                                                          | 210                                  | 50                         | 45                                      | 0.48                          | 1.7                                        | 77.4                                     | 29.9                                    |
| Example 8*  | 50                                                          | 210                                  | 43                         | 45                                      | 0.55                          | 52.8                                       | 56.8                                     | 29.2                                    |
| Example 9*  | 50                                                          | 210                                  | 33                         | 45                                      | 1.13                          | 54.5                                       | 51.7                                     | 28.2                                    |
| Example 10* | 30                                                          | 110                                  | 47                         | 45                                      | 2.04                          | 59.5                                       | 47.4                                     | 32.6                                    |
| Example 11* | 30                                                          | 110                                  | 35                         | 35                                      | 1.98                          | 62.6                                       | 46.5                                     | 28.8                                    |

The symbol \* represents a comparative example.

μm or smaller. A summed area (μm<sup>2</sup>) of the above crystals was obtained as an area of the vertically long crystal grains. That is, setting conditions of OIM Analysis 7 were shown as in Table 3.

TABLE 3

|                        |                                                                                |         |
|------------------------|--------------------------------------------------------------------------------|---------|
| Aspect ratio           | Aspect ratio of ellipse fit to grain                                           | <=0.5   |
| Gradient of major axis | Orientation (relative to the horizontal) of major axis of ellipse fit to grain | <=0.707 |
| sinθ *                 | in degrees                                                                     |         |
| Minor axis of ellipse  | Length of minor axis of ellipse fit to grain in microns                        | <=0.38  |

\*θ <= 45 and θ >= 135

—Calculation of Proportion of Vertically Long Crystals:

Using the area  $S_{vc}$  (μm<sup>2</sup>) of the vertically long crystal grains obtained in the primary extraction and the secondary extraction and an area  $S_{OA}$  (μm<sup>2</sup>) of the observation field, a proportion occupied by the vertically long crystal grains relative to the area occupied by the copper crystal grains was calculated with a formula of  $100 \times S_{vc} / S_{OA}$  to be specified as the proportion of the vertically long crystals (%). Table 4 shows results.

<Measurement of Original Tensile Strength>

A sample of the electrodeposited copper foil without annealing was cut in a size of 10 mm×100 mm to obtain a

The invention claimed is:

1. An electrodeposited copper foil having a ten-point average roughness  $Rz$  of 0.1 μm or larger and 2.0 μm or smaller on at least one surface,

wherein in cross-sectional analysis by electron backscatterer diffraction (EBSD), a proportion of an area occupied by copper crystal grains satisfying all of the following conditions:

i) (101) orientation;

ii) an aspect ratio of 0.500 or less;

iii)  $|\sin \theta|$  of 0.001 or more and 0.707 or less, where  $\theta$  (°) is an angle between a normal line of an electrode surface of the electrodeposited copper foil and a major axis of the copper crystal grain; and

iv) when the crystal is elliptically approximated, a length of a minor axis of 0.38 μm or smaller,

relative to an area of an observation field occupied by copper crystal grains is 63% or more.

2. The electrodeposited copper foil according to claim 1, wherein the electrodeposited copper foil has a ten-point average roughness  $Rz$  of 0.1 μm or larger and 2.0 μm or smaller on both surfaces.

3. The electrodeposited copper foil according to claim 1, wherein after annealing at 180° C. for 1 hour, the electrode-

posited copper foil has a tensile strength measured in accordance with IPC-TM-650 of 15 kgf/mm<sup>2</sup> or more and less than 25 kgf/mm<sup>2</sup>.

4. The electrodeposited copper foil according to claim 1, wherein in an unannealed original state, the electrodeposited copper foil has a tensile strength measured in accordance with IPC-TM-650 of 56 kgf/mm<sup>2</sup> or more and less than 65 kgf/mm<sup>2</sup>. 5

5. A flexible substrate, comprising the electrodeposited copper foil according to claim 1. 10

\* \* \* \* \*